

# UNITED STATES PATENT OFFICE.

FREDERICK M. BECKET, OF NIAGARA FALLS, NEW YORK, ASSIGNOR TO ELECTRO METALURGICAL COMPANY, A CORPORATION OF WEST VIRGINIA.

## PROCESS OF MAKING LOW-CARBON METALS OR ALLOYS.

No. 891,898.

Specification of Letters Patent.

Patented June 30, 1908.

Application filed August 24, 1905. Serial No. 275,667.

*To all whom it may concern:*

Be it known that I, FREDERICK M. BECKET, a subject of the King of Great Britain, residing at Niagara Falls, in the county of Niagara and State of New York, have invented certain new and useful Improvements in Processes of Making Low-Carbon Metals or Alloys, of which the following is a specification.

10 This invention is a process for the production of metals and alloys of low carbon content, and is more particularly applicable to the metals chromium, molybdenum, vanadium and tungsten and to the alloys of these 15 metals with iron or nickel.

The invention consists in first producing from a suitable ore an alloy high in silicon and low in carbon, and thereafter eliminating all or part of the silicon by reacting upon 20 further quantities of ore.

As is well known, the presence of carbon is undesirable in the various metals and alloys such as ferro-chromium, ferro-tungsten, etc., which are used for imparting special properties to steel, and the value of these alloys increases greatly as their carbon content decreases. With the object of producing metals and alloys of low carbon content many processes have been devised in which reducing agents other than carbon are employed, such reducing agents being, however, very costly. Processes have also been devised in which a high carbon alloy is produced and thereafter subjected in a secondary stage to 25 the refining action of various decarburizing agents which are also either costly or cause large losses of the metal produced in the first stage.

According to my invention an economical 40 process is provided for the production of the above mentioned metals and alloys with a content of carbon and silicon which may be easily controlled.

I have found that if the oxids or oxygen 45 containing compounds of chromium, molybdenum, vanadium or tungsten are mixed with varying quantities of silicious material and subjected to the reducing action of carbon, the resulting product containing the metals 50 chromium, molybdenum, vanadium, tungsten or their alloys, contains silicon and carbon in varying proportion, the percentage of carbon being lower as the percentage of silicon is higher; I have also found that by in-

corporating silicious material and carbon in 55 the charge in certain proportions it is possible to produce these metals and alloys containing a very small proportion of carbon. I have also found that if the products made in the manner just described are suitably treated with a new supply of ores or compounds of the desired metals, the silicon may be practically eliminated and the carbon content still further diminished.

In order that my invention may be fully 65 understood I shall describe its application to the manufacture of low carbon ferro-chromium, it being understood that this alloy is typical only of those heretofore mentioned.

As a source of chromium and iron I generally 70 use the mineral chromite containing from 50 to 52 percent. chromium sesquioxid,  $\text{Cr}_2\text{O}_3$ , and from 16 to 17 percent. ferrous oxid,  $\text{FeO}$ . With chromite I mix a quantity of sand or other silicious material, sufficient carbon to 75 reduce not only the oxids of chromium and of iron but also a part or all of the silicious material, and a flux, such as lime, to form a suitable slag with the impurities generally existing in the chromite and with any portion of 80 the silicious material which may be unreduced. This mixture is then subjected to a high temperature by means of electrically developed heat and yields an alloy containing chromium, iron, silicon and a small percent- 85 age of carbon. This is the first stage of my process. The second stage consists in treating the alloy thus produced, preferably in another electric furnace which when a very low carbon product is desired should have a 90 hearth of material other than carbon, with a mixture of chromite or other suitable oxid ore and any fluxing material such as lime.

As a result of this treatment the silicon of the 95 alloy produced in the first stage of the process combines with the oxygen of the oxids contained in the chromite or other ore and forms silica which passes into the slag, an equivalent proportion of chromium and iron being reduced and accumulating with the chro-

mium and iron produced in the first stage. As one pound of silicon will liberate from the 100 oxid of chromium,  $\text{Cr}_2\text{O}_3$ , 2.44 pounds of chromium, and as this same quantity of silicon will liberate from the oxid of iron,  $\text{FeO}$ ,

105 3.9 pounds of iron, it will be understood that the silicon in the alloy produced in the first stage is replaced by a greater weight of

chromium and iron, and that therefore the percentage of carbon in the finished product may be further reduced.

The proportions of carbon and silica incorporated with a given quantity of chromite to be smelted in the first stage of my process depend upon the quality of the chromite and the percentage of carbon which it is desired the finished ferro-chromium should contain.

5 To make a ferro-chromium containing about one percent. carbon from chromite of the quality above referred to, I have found that the charge may advantageously consist of equal parts by weight of chromite, sand and ordinary coke. The alloy obtained when this charge is smelted in the electric furnace has approximately the following analysis: chromium 51.3%; iron 17.5%; silicon 30.0%; carbon 1.2%. In the second stage of the process this alloy is treated in the electric furnace with a new supply of chromite in the proportion of about six pounds of chromite to every pound of silicon in the alloy, this proportion of chromite to silicon being very 10 slightly in excess of that theoretically necessary to supply sufficient oxygen for the conversion of the silicon to silica. As a result of this treatment the silicon is practically eliminated, and more chromium and iron have 15 been produced, and the alloy will now analyze practically as follows: chromium 70.0%; iron 28.9%; carbon 1.0%; silicon 0.10%. If an alloy of even lower carbon content is required, a higher percentage of silicon is obtained in the metallic products from the first 20 stage of the process by using an increased proportion of both sand and coke to chromite, with the result that the carbon content is still lower. Similarly by using a lower proportion of sand and coke, metallic products containing less silicon and more carbon are obtained. It will be seen that by thus controlling, in the first stage of the process, the 25 carbon content of the alloy, the percentage of carbon in the finished product may be controlled within very narrow limits.

In order to obtain satisfactory results with the metals named it is practically necessary that the first stage of the process should be 30 carried out at the high temperature of the electric furnace, and it is preferred that the second or refining stage should also be carried out in the same or other electric furnace. To obtain the advantages of continuous operation and in general to conduct the process in the most advantageous manner I prefer to employ two electric furnaces in close proximity to each other, so that the metal or alloy containing considerable silicon produced 35 in one furnace may be tapped directly into the other furnace, in which the second stage of the process is carried out and from which the finished products are tapped as desired. By this method the total electrical energy 40 consumed in the process is less than when the

metallic products of one furnace are allowed to cool before treatment in the same or other furnace.

In the production of chromium, molybdenum, vanadium, tungsten or alloys of 45 these metals in the electric furnace it is known that if sufficient carbon is used in the charge to obtain a high yield of these metals from the quantity of ore furnace, the resulting metallic products contain a relatively high proportion of carbon; and as is commonly practiced, if less than the theoretical quantity of carbon is supplied to the charge, poor yields are obtained and the carbon or graphite in the very expensive 50 form of electrodes is rapidly consumed. Referring to the above example of production of ferro-chromium, had the silicious material not been used in the charge and had the theoretical quantity, or slight excess of carbon, been employed, the carbon in the resulting product would have been about 8-10 percent. Had considerably less than the theoretical carbon been used in the charge, the resulting ferro-chromium 55 would have contained 4-6 percent. carbon. One of the advantages of my process lies in the possibility of using almost any excess of carbon as a reducing agent in the charge employed in the first stage, thereby obtaining very high yields of the desired metals and causing a great saving in consumption of carbon or graphite electrodes. As a further advantage I have found it possible to produce low carbon, high silicon products in 60 an electric furnace in which not only the side walls but the hearth on which the metal rests during the first stage of the process are made of the cheap and durable material carbon. As other advantages it may be pointed out that 65 ores which are usually considered as low grade on account of the presence of undue proportions of silica, and which are therefore considered unfit for the manufacture of the specified metals or alloys, can be successfully and economically used in this process. The same remark applies to the purity of the carbonaceous reducing agents such as coke. When the ores contain sufficient silica 70 for the purpose, no addition of silicious material is required, and it is then only necessary to so proportion the coke that the desired amount of silicon is obtained. This is the case when low carbon ferro-vanadium is produced from vanadiferous sandstone.

As the reaction between silicon and the metallic oxides employed is strongly exothermic, a relatively very small amount of electrical energy is required to eliminate the silicon in the second stage of the process 75 with the production of a further quantity of the desired metals almost equivalent to that theoretically possible with a given amount of silicon. The silicon can readily be so far eliminated that the final product 80

contains not more than five or six one-hundredths of one percent of silicon; or if it be desired to produce a product containing any given percentage of silicon this may be done by properly proportioning the quantity of chromite.

I claim:

1. The process of producing low carbon metals or alloys which consists in producing under electric furnace conditions a metallic product low in carbon and high in silicon, and then oxidizing part or all of the silicon, substantially as described.

2. The process of producing low carbon metals or alloys which consists in reacting under electric furnace conditions with carbon on a charge containing an oxid ore and silica to produce a metallic product low in carbon and high in silicon, and then oxidizing part or all of the silicon, substantially as described.

3. The process of producing low carbon metals or alloys which consists in producing under electric furnace conditions a metallic product low in carbon and high in silicon and then reacting on said product with an oxid ore to oxidize the silicon, substantially as described.

4. The process of producing low carbon metals or alloys which consists in reacting under electric furnace conditions with carbon

on a charge containing an oxid ore and silica to produce a metallic product low in carbon and high in silicon, and then reacting on said product with additional quantities of the same oxid ore to oxidize silicon, substantially as described.

5. The process of producing low-carbon ferrochrome, which consists in reacting under electric furnace conditions with carbon on a charge containing an oxid ore of chromium and silica to produce a metallic product low in carbon and high in chromium and silicon, and then oxidizing part or all of the silicon, substantially as described.

6. The process of producing low-carbon ferrochrome, which consists in reacting under electric furnace conditions with carbon on a charge containing an oxid ore of chromium and silica to produce a metallic product low in carbon and high in chromium and silicon, and then reacting on said product with additional quantities of the same oxid ore to oxidize silicon, substantially as described.

In testimony whereof, I affix my signature in presence of two witnesses.

FREDERICK M. BECKET.

Witnesses:

JASPER WHITING,  
Wm. L. HEIM.